

# United States Patent

[11] 3,617,435

[72] Inventor **John H. Kalisch**  
**Hawkesbury, Ontario, Canada**  
[21] Appl. No. **734,044**  
[22] Filed **June 3, 1968**  
[45] Patented **Nov. 2, 1971**  
[73] Assignee **Canadian International Paper Company**  
**Montreal, Ontario, Canada**  
**Continuation-in-part of application Ser. No.**  
**539,683, Apr. 4, 1966, now Patent No.**  
**3,479,249.**  
**The portion of the term of the patent**  
**subsequent to Nov. 18, 1986, has been**  
**disclaimed.**

[54] **TREATMENT OF WOODPULP WITH AN  
ALKALINE SOLUTION CONTAINING  
FORMALDEHYDE PRIOR TO A BISULFITE  
COOKING THEREOF**  
**8 Claims, 5 Drawing Figs.**  
[52] U.S. Cl..... **162/72,**  
..... **162/83, 162/84, 162/86**

[51] Int. Cl..... **D21c 3/20**  
[50] Field of Search..... **162/9, 17,**  
..... **18, 24, 25, 26, 32, 72, 83, 84, 86, 165, 166, 180**

[56] **References Cited**  
**UNITED STATES PATENTS**  
2,885,317 5/1959 Collin et al. .... **162/84 X**  
2,904,460 9/1959 Nolan..... **162/86 X**  
3,124,503 3/1964 Zachariasen ..... **162/9**  
3,479,249 11/1969 Kalisch..... **162/72 X**

*Primary Examiner—S. Leon Bashore*  
*Assistant Examiner—Arthur L. Corbin*  
*Attorney—R. G. McClenahan*

**ABSTRACT:** A bisulfite wood-pulping process in which not more than about 2 percent by weight, based on the wood, of formaldehyde in an alkaline solution is used to pretreat the wood prior to the bisulfite cooking.

SHEET 1 OF 4

FIG. 1



FIG. 2

INVENTOR.  
JOHN H. KALISCH

BY

*John H. Kalisch*

ATTORNEY

FIG. 3



FIG. 4

| PULP DATA                      | COOKING PROCESS |        |        |        | E      |
|--------------------------------|-----------------|--------|--------|--------|--------|
|                                | A               | B      | C      | D      |        |
| TOTAL COOKING TIME, HOURS      | 12.20           | 9      | 8      | 8 1/2  | 6      |
| SCREENED YIELD, % O.W.         | 51.4            | 58.3   | 59.7   | 60.5   | -----  |
| SCREENINGS, % O.W.             | 0.7             | 0.75   | 1.2    | 2.0    | -----  |
| TOTAL YIELD, %                 | 52.1            | 59.05  | 60.9   | 62.05  | 76.03* |
| BRIGHTNESS (ELREPHO) %         | 63.7            | 62.0   | 59.7   | 58.5   | 60.2   |
| ROE NUMBER                     | 6.3             | 9.4    | 9.4    | 12.1   | 27.0   |
| K#                             | 23              | 40.6   | 48.7   | 68.3   | 122    |
| VISCOSITY, TAPPI 230 Sm 50, cP | 28.8            | 32.6   | 27.7   | 21.3   | N.D.   |
| ALPHA CELLULOSE, %             | 85.9            | 86.2   | 87.0   | 86.9   | 88.3   |
| PENTOSAN, %                    | 5.0             | 5.1    | 5.3    | 5.1    | 4.8    |
| MANNAN, %                      | 16.5            | 13.3   | 13.9   | 14.4   | 15.9   |
| XYLAN, %                       | 4.8             | 4.3    | 4.2    | 4.5    | 5.3    |
| RESIN, %                       | 0.47            | 0.5    | 0.4    | 0.5    | 0.57   |
| LIGNIN, %                      | 2.0             | 3.6    | 6.7    | 7.8    | 17.7   |
| STRENGTH AT CSS, ml :          |                 |        |        |        |        |
| MULLEN, % PTS/LB               | 133             | 140    | 141    | 145    | 132    |
| BREAKING LENGTH, m.            | 11,200          | 11,100 | 11,300 | 11,100 | 11,300 |
| TEAR FACTOR                    | 71              | 61     | 64     | 61     | 59     |
| FOLD (SCHOPPER)                | 500             | 470    | 350    | 340    | 400    |
| OPACITY, %                     | 63.9            | 56.6   | 62     | 59     | 61.0   |
|                                |                 |        |        |        | 56.5   |
|                                |                 |        |        |        | 68     |
|                                |                 |        |        |        | 62.7   |
|                                |                 |        |        |        | 69.0   |
|                                |                 |        |        |        | 66.0   |

\*OBTAINED BY DISC REFINING OF WHOLE COOK.

FIG. 5

| PULP DATA                      |        | COOKING PROCESS |       |        |        |
|--------------------------------|--------|-----------------|-------|--------|--------|
|                                |        | F               | G     | H      | I      |
| TOTAL COOKING TIME, HOURS      |        |                 | 7:30  |        | 6:55   |
| SCREENED YIELD, % O.W.         |        |                 |       |        |        |
| SCREENINGS, % O.W.             |        |                 |       |        |        |
| TOTAL YIELD, %                 | 49.3*  |                 | 60.6* | 70.0*  | 74.6*  |
| BRIGHTNESS (ELREPHO) %         | 50.6   |                 | 54.7  | 54.3   | 54.7   |
| ROE NUMBER                     | 8.4    |                 | 17.5  | 27.6   | 28.8   |
| K#                             | 40     |                 | 85    | 125    | 130    |
| VISCOOSITY, TAPPI 230 Sm50, CP | 22.3   |                 | 88.6  | 87.6   | 88.5   |
| ALPHA CELLULOSE, %             |        |                 | 5.18  | 4.79   | 5.18   |
| PENTOSAN, %                    | 4.4    |                 |       |        |        |
| MANNAN, %                      |        |                 |       |        |        |
| XYLAN, %                       |        |                 |       |        |        |
| RESIN, %                       | 0.59   |                 | 0.63  | 0.56   | 0.45   |
| LIGNIN, %                      | 10.1   |                 |       | 19.6   | 21.5   |
| STRENGTH AT CSF, m:            |        |                 |       |        |        |
| MULLEN, % PTS/LB               | 391    | 300             | 378   | 500    | 500    |
| BREAKING LENGTH, m             | 146    | 158             | 139   | 132    | 144    |
| TEAR FACTOR                    | 12,328 | 12,900          | ---   | 11,508 | 10,700 |
| FOLD (SCHOPPER)                | 65     | 66              | 69    | 69     | 62     |
| OPACITY, %                     | 514    | 570             | 383   | 270    | 280    |
|                                | 62.9   | 60.5            | 66.6  | 70     | 64     |
|                                |        |                 |       | 70     | 70     |

\*OBTAINED BY DISC REFINING OF WHOLE COOK.

**TREATMENT OF WOODPULP WITH AN ALKALINE  
SOLUTION CONTAINING FORMALDEHYDE PRIOR TO  
A BISULFITE COOKING THEREOF**

This application is a continuation-in-part of copending U.S. Ser. No. 539,683, filed Apr. 4, 1966 now issued to U.S. Pat. No. 3,479,349.

That patent relates to a wood-pulping process for making paper pulps of improved unbleached brightness, increased yield, and other improved pulp characteristics. More particularly, it relates to the use of an alkaline solution containing a low concentration of formaldehyde before cooking wood by the sulfite process. The use of this process is highly advantageous for coniferous woods and, particularly, for woods such as pines in which the polyphenolic components interfere with normal pulping by the sulfite process. The sulfite process is discussed at length in, for instance, Calkin, J.B.; *Modern Pulp and Paper Making*: (3rd Ed.) Reinhold Publishing Corporation; New York, 1957; p. 81 et seq.

Many attempts have been made in the past to arrive at a satisfactory process for pulping of pines by the sulfite process. The use of soluble bases such as sodium, magnesium, and ammonium has led to substantial improvements over calcium base booking. Pine chips from young trees can be successfully cooked by the conventional calcium base sulfite process, but difficulties increase with the age of the tree. The need to harvest relatively older trees from slower growing northern pines in contrast to fast-growing southern pine indicates the problem.

It has been shown that the heartwood portion of pines is responsible for their more difficult pulping characteristics; sapwood, on the other hand, pulps satisfactorily with any base by the sulfite process. Consequently, the relatively high proportion of heartwood in slow-growing trees of normal age for harvesting eliminates the use of calcium base in conventional sulfite cooking.

However, even the use of a soluble base in pulping of pines will result in pulp characteristics inferior to those of spruce and other coniferous woods of relatively low resin content. This is particularly apparent with reference to delignification (yield at comparable Roe number) and unbleached pulp brightness.

Hägglund (Cellulose Chemie 8 (No. 3 25 (1927)) and more recently Erdtmann (Tappi 23, 303 (1949)) have shown that an ether-, benzene-insoluble, but alcohol- or acetone-soluble compound contained in the heartwood of pines interferes with normal delignification in lime base sulfite cooking. Such compounds were identified by Erdtmann as resorcinol-like polyphenols such as pinosylvin, pinosylvin methyl ether, and flavanones which amount to about 20 percent of the total resin of pine or to approximately 1 percent of the heartwood portion of pine. Polyphenols condense easily with lignin at higher temperature. As a result, large lignin-polyphenol complexes are formed with simultaneous blocking of active groups which are needed for sulfonation and final solubilization of the lignin.

Blocking of the reactive position of the polyphenol prior to the start of the sulfite cook is needed to prevent condensation with lignin. Experiments by Alder and Stockman (Svensk Papperst. 54,477 (1951)) with phenolic model compounds (catechol) indicated that such a reaction will occur with formaldehyde in an alkaline medium so that a hydroxybenzyl alcohol is formed according to the Lederer-Manasse reaction. This hydroxybenzyl alcohol reacts with sulfite and forms a hydroxybenzyl sulfonic acid. The following illustrates the above-mentioned reactions:



The above-noted investigators attempted to apply their concept to sulfite pulping of pine heartwood by pretreating it with a relatively concentrated solution of formaldehyde (20 percent concentration) in an alkaline (0.1 N NaOH) or aqueous solution at elevated temperature (80° C.) for 6 hours. Pulp made by this procedure showed greatly improved yield, but was still not satisfactory owing to low brightness (discoloration) as well as shiviness.

A process overcoming the deficiencies in the treatments just discussed is described in copending U.S. application Ser. No. 539,683 filed Apr. 4, 1966. This process is based on the discovery that, in contrast to previously described findings, considerable improvements not only in the pulping of pines, but also of other coniferous woods such as spruce, occur if the pretreatment of the pine chips is carried out both at a low temperature and at a low concentration of formaldehyde in alkali. Impregnation temperatures preferably below about 5° C. and formaldehyde concentrations between about 0.15 and 0.4 percent, corresponding to 0.75 percent to 2.0 percent (added) by weight based on wood at an alkali solution-to-wood ratio of 5:1 by weight, result in highly significant improvements. Such process is denominated the AFS-process, and is distinguished from the so-called ACSNa and AS-processes in the copending application. (AFS=Alkaline formaldehyde pretreatment followed by sulfite pulping; ACSNa=acid sulfite pulping with sodium base; and, AS=alkali pretreatment followed by sulfite pulping.)

The low formaldehyde concentration and the low impregnation temperature promote the reaction of pinosylvin and other polyphenolic compounds according to the Lederer-Manasse reaction and substantially slow or prevent the otherwise competing, but undesired lignin-formaldehyde condensation, which proceeds disadvantageously at an increased speed at a higher concentration of formaldehyde and at a higher temperature.

Experimental results on jack pine presented in the above-noted, copending application show that unbleached pulp yield, brightness, and viscosity are increased by the alkaline formaldehyde pretreatment, reaching maxima between 2 and 4 percent formaldehyde. All these properties decrease as temperature is increased above about 40°-50° C.

AFS-jack pine pulp in comparison with a conventional soda base sulfite pulp shows 9 points gain in brightness and a 5 percent actual gain in screened pulp yield. Corresponding gains for AFS-black spruce pulp are a 7-point gain in brightness and 6 percent actual increase in screened pulp yield. AFS-Douglas fir showed a 3 percent higher actual yield and 12.5-point gain in brightness in comparison with the corresponding AcSNa pulp. Other properties, such as high viscosity and high mannan content, reflect the unique characteristics of pulps from alkali-formaldehyde pretreated wood.

Paper strength tests of AFS pulps showed that they are equal to conventional sulfite pulps at a freeness of 300 CSF, but surpass them at a freeness of 100 CSF. Consequently, such pulps make very satisfactory paper pulps both for unbleached and bleached grades, but are particularly suitable for glassine-type pulps as a result of fast beating and good retention of strength in beating to low freeness.

It has now been found that the alkaline formaldehyde pretreatment gives similar or even greater advantages when used in connection with the bisulfite cooking process, so denominated because base and sulfur dioxide are present in the stoichiometrical proportions to give only the bisulfite, without excess of either constituent. The complete operation is here referred to as the AFB process.

AFB cooking conditions are obtained by treating NaOH-CH<sub>2</sub>O-impregnated chips with an aqueous sulfuric acid solution which contains the amount of SO<sub>2</sub> required to produce sodium bisulfite instead of the free-SO<sub>2</sub> required to produce sodium bisulfite instead of the free-SO<sub>2</sub>-containing sodium acid sulfite liquor. Instead of the aqueous solution, liquid SO<sub>2</sub> may be employed, the choice depending largely on local availability.

Bisulfite is formed stoichiometrically according to the following equation:



This reaction should lead to pH 4. However, in practice it has been found that the actual quantity of  $\text{SO}_2$  should be about 2 to 8 percent less than the theoretically calculated one. This has been found desirable in order to prevent a substantial lowering in pH (resulting from wood acids produced during cooking) below the bisulfite range.

The general method of the present invention is as follows:

A blend, for instance, of balsam-spruce chips is treated with a sodium hydroxide solution containing a small quantity of formaldehyde. The liquor is drained after the required time of impregnation. The amount of NaOH taken up by the chips is determined by measuring both volumes and NaOH contents of the fresh liquor added and the drained liquor recovered. The amount of  $\text{SO}_2$  required to form bisulfite is calculated less 6 percent based on equation (1) and a sulfurous acid solution containing the required quantity of  $\text{SO}_2$  is injected into the digester. A cold pH preferably between 3 and 4 will be reached after a few hours of cooking. It should also be understood that the time-temperature cooking chart used is designed to allow for ample diffusion time of chemicals from the outside of the chips toward the center and vice versa before a substantial temperature rise occurs.

For a clearer understanding of the present invention, reference should be had to the following example:

#### example 1

[Wood: Balsam-spruce mill chips (10,500 g. oven-dry weight)]

##### Caustic impregnation

| Liquor:                             | NaOH, grams/litre | 50 | 35 |
|-------------------------------------|-------------------|----|----|
| $\text{CH}_2\text{O}$ , grams/litre | 4                 |    |    |
| Volume added, liters                | 54                |    |    |
| Temperature, °C                     | 26                |    |    |
| Liquor to wood ratio                | 6.1:1             |    |    |
| Pressure, p.s.i.                    | 100               |    |    |
| NaOH take-up, g.                    | 1,167             |    |    |

##### Bisulfite cook

| Liquor:                      | Sulfurous acid, $\text{SO}_2$ , percent | 4.12 | Time, hours     | 0  | 1  | 2  | 3   | 4   | 5   | 6   |
|------------------------------|-----------------------------------------|------|-----------------|----|----|----|-----|-----|-----|-----|
| Volume added, liters         | 44.4                                    |      | Temperature, °C | RT | 40 | 50 | 90  | 125 | 150 | 155 |
| $\text{SO}_2$ content, grams | 1,185                                   |      | Pressure        | 90 | 90 | 85 | 110 | 90  | 90  | 90  |
| pH                           | 3.5                                     |      |                 |    |    |    |     |     |     |     |
| Liquor to wood ratio         | 4.2                                     |      |                 |    |    |    |     |     |     |     |
| Max. cooking temperature, °C | 155                                     | 45   |                 |    |    |    |     |     |     |     |
| Pressure, p.s.i.g            | 285                                     |      |                 |    |    |    |     |     |     |     |

<sup>1</sup> 30 grams less than that required for complete formation of  $\text{NaHSO}_3$ .

<sup>2</sup> Constant from start to finish.

##### COOKING CHART

| Time, hours              | 0    | 1    | 2    | 3    | 4    | 5    | 6    | 7    | 8    | 8½   |
|--------------------------|------|------|------|------|------|------|------|------|------|------|
| Temp., °C                | 25   | 40   | 50   | 90   | 125  | 155  | 155  | 155  | 155  | 155  |
| Pressure, p.s.i.g        | 85   | 44.4 |      |      |      |      |      |      |      |      |
| Total $\text{SO}_2$ %    | 3.06 | 2.85 | 2.7  | 2.6  | 2.58 | 2.10 | 1.54 | 1.06 | 0.76 | 0.66 |
| Combined $\text{SO}_2$ % | 0.96 | 1.16 | 1.2  | 1.19 | 1.18 | 0.9  | 0.64 | 0.46 | 0.32 | 0.28 |
| Cold pH                  | 2.1  | 2.5  | 2.86 | 2.70 | 2.75 | 2.90 | 3.10 | 3.40 | 3.5  | 3.45 |

It should be understood that variations of the procedure of the example such as, for instance, caustic impregnation with lower concentrations of NaOH and  $\text{CH}_2\text{O}$  also produce satisfactory results. Furthermore, other caustic impregnation media including the strongly alkaline carbonates of such bases or a combination of carbonates with alkalies are within the scope of this invention, and indeed have certain advantages which will be discussed later.

Results produced in accordance with the AFB process of the present invention are shown in FIG. 4 (table 1a) and are compared with four conventional sodium bisulfite process (pH 4) controls reported in FIG. 5 (table 1b). For simplicity, such conventional process is designated therein as the BSNa process. The same spruce-balsam blend was used in all cases.

It should be noted that AFB high-yield pulps were obtained, with one exception, as screenable pulps without the need of mechanical refining. In contrast, the conventional bisulfite pulps required mechanical refining.

Advantages of AFB pulps over conventional bisulfite pulps

are the following:

1. Screened pulp yields of about 60 percent without mechanical refining (this is due to better delignification and higher retention of hemicelluloses);
  2. Pulps at yields above 60 percent and up to 75 percent can be obtained by mild refining in a single-pass operation;
  3. Considerably higher unbleached brightness; and,
  4. Good strength characteristics except somewhat lower tear and opacity.
- 5 The new AFB pulps are particularly valuable as a replacement for ordinary unbleached sulfite pulps, especially whenever higher brightness and high screened yield and good beatability are desired, as in newsprint or publication grade papers.
- 10 15 Replacement of NaOH with  $\text{Na}_2\text{CO}_3$  or, preferably, a combination of  $\text{Na}_2\text{CO}_3$  with NaOH in the impregnation stage of AFB cooking has been found to contribute further significant improvements in delignification, paper strength characteristics, and the brightness of AFB pulps. The following example illustrates such a cooking procedure and sets forth pulp data:

#### EXAMPLE 2

Conventional spruce-balsam mill chips were impregnated with a solution of 80 g.  $\text{Na}_2\text{CO}_3$ , 11 g. NaOH and 2.8 g.  $\text{CH}_2\text{O}$  per liter, at R.T. and 100 p.s.i. for 90 minutes at a liquor-to-wood ratio of 5:1. Three pressure cycles of 1 minute each were applied to improve liquor penetration. The liquor was then drained and an aqueous  $\text{SO}_2$  solution was injected, containing the amount of  $\text{SO}_2$  necessary to convert the base into sodium bisulfite according to the following reactions:



Cooking was carried out according to the following chart for a total time of 6 hours, 5 minutes:

| Time, hours     | 0  | 1  | 2  | 3   | 4   | 5   | 6   |
|-----------------|----|----|----|-----|-----|-----|-----|
| Temperature, °C | RT | 40 | 50 | 90  | 125 | 150 | 155 |
| Pressure        | 90 | 90 | 85 | 110 | 90  | 90  | 90  |

The liquor-to-wood ratio was 4:1 using a full digester and maintaining 90 p.s.i. throughout the cook. The cooked chips were given a mild mechanical refining treatment. The above

conditions produced the following pulp:

| Pulp Yield          | Strength (PFI Mill) |                      |        |  |  |  |
|---------------------|---------------------|----------------------|--------|--|--|--|
|                     | at 500 CSF:         |                      |        |  |  |  |
| Brightness, % (Elr) | 59                  | Mullen, % pts./lb.   | 140    |  |  |  |
| Kappa number        | 95                  | Tensile strength, m. | 12,500 |  |  |  |
| Roc number          | 21.4                | Tear Factor          | 70     |  |  |  |
|                     |                     | Fold (Schopper)      | 210    |  |  |  |
|                     |                     | Opacity, %           | 64     |  |  |  |

The following table shows pulp data for the two variations (i.e.,  $\text{NaOH} + \text{CH}_2\text{O}$  and  $\text{Na}_2\text{CO}_3 + \text{NaOH} + \text{CH}_2\text{O}$ ) of the AFB process and comparative data for a conventional sodium bisulfite (BSNa) control cook. All data were extrapolated to 75 percent pulp yield for easier comparison:

| Pulp Yield: 75% | AFB | PULP DATA  | $\text{Na}_2\text{CO}_3 + \text{NaOH}$ | NaOH | BSNa |
|-----------------|-----|------------|----------------------------------------|------|------|
|                 |     | Roc number | 23.9                                   | 26.0 | 31.0 |

Table - Continued

|                         |        |        |        |
|-------------------------|--------|--------|--------|
| Brightness, % (Elr)     | 60.0   | 58.5   | 56     |
| PFI Strength at 500 CSF | 143    | 124    | 140    |
| Mullen, % pts./lb.      |        |        |        |
| Breaking Length, m.     | 12,500 | 10,300 | 11,800 |
| Tear Factor             | 67     | 63     | 63     |
| Mannan, %               | 15.7   | 13.7   | 11.8   |

FIGS. 1, 2 and 3 give the same comparison for Roe number, brightness and breaking length over a range of pulp yields.

The reaction between carbonate and also hydroxide with  $\text{SO}_2$  proceeds primarily within the chip. The pH gradually decreases,  $\text{CO}_2$  being generated until the formation of sodium bisulfite is completed. The initial pH during caustic impregnation is 12.5; however, decomposition of the carbonate starts below pH 8.5. Theoretically, for each mol (106 grams) of  $\text{Na}_2\text{CO}_3$ , 1 mol of  $\text{CO}_2$  (44 grams or 22.4 liters at 0° C., 760 mm.) is formed. The solubility of  $\text{CO}_2$  in water at a pressure of 80 p.s.i. and 30° C. is 0.4 gram  $\text{CO}_2$ /100 ml.  $\text{H}_2\text{O}$ . This will lower pH to 3.5. Therefore, this system containing excess  $\text{CO}_2$  and carbonic acid is in a position to exert effectively within the chip a buffering action and, perhaps, also other not yet completely understood reactions during the initial stages of the bisulfite cook. It is suggested that the above-indicated effects are a contributing or even major factor in the striking improvement in pulp characteristics.

In the AFB process, as in the AFS process of copending U.S. application Ser. No. 539,683, alkaline impregnation at a hydrostatic pressure of 100 p.s.i.g. and at temperatures below 50° C. requires 90 minutes for uniform penetration of chips. If impregnation temperatures above 50° C. are applied, a significant lowering in both brightness and delignification rate occurs. Furthermore, it has been found that the conversion from alkaline to acid (bi) sulfite condition within the chips (which is controlled by a relatively slow diffusion) must be completed (requiring 90 minutes at 50° C. and 100 p.s.i.g.) before the chips can be subjected to higher cooking temperatures. Such measures are necessary to prevent the inactivation of lignin in an alkaline medium with its detrimental effects on the subsequent bisulfite cooking stage. The necessity for the above conditions has heretofore limited the AFS and AFB processes to slow batch cooking.

However, it has been discovered that the above limitations imposed by times and temperatures can be resolved by conducting both the caustic and the acid stages at pressures substantially above the 100 p.s.i.g. mentioned previously. Pressures in the neighborhood of 200 p.s.i.g. have been found adequate. Improvement levels off above this point although higher pressures may be used if desired. This modification shortens the  $\text{Na}_2\text{CO}_3+\text{NaOH}+\text{CH}_2\text{O}$  impregnation stage to a fraction of the previously required time, a few minutes only, and it also permits a rapid and complete conversion of the chemicals within the chip from an alkaline to an acid condition. Be it noted, however that the temperature employed in the impregnation should be kept as low as possible. With the short impregnation time (about 2 minutes) made possibly by use of 200 p.s.i.g. pressure, the upper limit should be about 100° C.

It has also been discovered that, as a result of the short exposure time to an alkaline environment, the otherwise detrimental effects of even moderately increased temperatures were no longer harmful. As a result of this, the previously imposed temperature restrictions and time requirements can be so modified as to make this process suitable for continuous pulping.

The following is a description of the principal features of a quick AFB process suitable for continuous operation:

Mill chips such as jack pine, spruce, balsam or blends are pretreated with an alkaline solution containing a mixture of sodium hydroxide, sodium carbonate, and formaldehyde, total  $\text{Na}_2\text{O}$  content 55 grams per liter, the proportion of carbonate being such that the  $\text{CO}_2$  liberated during the subsequent acidification step will assist in holding the pressure at the level of the impregnation step, i.e. about 200 p.s.i.g. or above, while avoiding an excess of  $\text{CO}_2$  which would have to be gotten rid of.

The composition of the caustic impregnation liquor must be adjusted in such a way that the combined strength of  $\text{Na}_2\text{CO}_3$  and NaOH is sufficient to result in a minimum takeup of about 10 percent  $\text{Na}_2\text{O}$  on wood. The concentration of NaOH in the  $\text{Na}_2\text{CO}_3$ -containing liquor must be adequate to obtain a minimum pH of 12.6.

For practical application 80 to 100 grams  $\text{Na}_2\text{CO}_3$  per liter and 11 to 5 grams NaOH per liter will satisfy the above requirement and also insure the desired pressures from the beginning of the cook. Lower amounts of  $\text{Na}_2\text{CO}_3$  and correspondingly higher levels of NaOH can be used as long as the desired level of  $\text{Na}_2\text{O}$  on wood and the required pressure buildup are obtained.

If the carbonate content is reduced below a level necessary to liberate sufficient  $\text{CO}_2$  to maintain the pressure required for quick conversion to sulfite after the impregnation stage, other means of pressure generation must be provided. Continuous pulping with two sequential stages prevents the use of a full digester which would be necessary for the use of a booster pump to maintain pressure. However, adequate pressure can easily and cheaply be maintained by, for instance, an oil-burning inert gas generator-compressor combination as commonly used for inert gas padding. But it should be kept in mind that, aside from pressurizing, carbonate has a beneficial effect on pulp properties, as described previously.

The level of formaldehyde in the impregnation liquor chosen will depend on the wood species used. The upper limit of formaldehyde is 2 percent by weight, based on the wood (or 0.4 percent by weight of the liquor, based on a liquor-to-wood ratio of 5 to 1). Woods containing objectionable resins such as jack pine, will require between 1 and 2 grams of  $\text{CH}_2$  (100 percent) per liter. On the other hand, less refractory woods such as balsam and spruce or blends can be adequately treated with liquors containing 0.25 to 0.5 grams  $\text{CH}_2\text{O}$  per liter. In making some pulp grades from these more readily pulped woods, the addition of even this small amount may not be economically justified—this will have to be decided by the requirements of the particular pulp grade and the current price of formaldehyde.

The impregnation liquor is applied at a liquor-to-wood ratio of 5 to 1 by weight and at a temperature between 20° C. and 50° C. and a pH of 12.8. The wood chips in the liquor are subjected to a hydrostatic pressure between 200 and 300 p.s.i.g. for 2 to 15 minutes. The impregnation liquor is then drained and made up to strength with  $\text{Na}_2\text{CO}_3$  and NaOH (and  $\text{CH}_2\text{O}$ ) for reuse in the next cook. After draining of the alkaline solution, water and liquid sulfur dioxide or an aqueous solution of sulfur dioxide is injected, so that a liquor-to-wood ratio of 4.5 to 1 is obtained. The temperature is then increased within 1 to 2 minutes to between 50° C. and a maximum of 100° C. The required quantity of sulfur dioxide is calculated to convert the alkali taken up by the wood into sodium bisulfite. Liberation of carbon dioxide from the ensuing reaction between  $\text{Na}_2\text{CO}_3$  and  $\text{SO}_2$  in the digester is regulated by pressure relief in such a manner as to maintain a constant pressure of at least 200 p.s.i.g. throughout the cook. As mentioned above, the required pressure may be obtained in whole or in part from a compressor-inert gas generator combination.

The following cooking chart is used:

|                    |       |     |     |           |
|--------------------|-------|-----|-----|-----------|
| Time Minutes       | 0     | 3   | 63  | 83        |
| Temp., °C.         | 20-50 | 100 | 100 | 155 (max) |
| Pressure, p.s.i.g. | 200   | 200 | 200 | 200 (max) |

Total cooking times vary between 2 and 3 hours depending on the desired Roe number or pulp yield.

It should also be mentioned that the process of the present invention can be carried out as a full or partial vapor phase (trickle phase) process with all its inherent advantages owing to savings in steam and a further reduction in cooking time.

In this case, only liquid  $\text{SO}_2$  and steam are admitted into the digester.

The method of the present invention is particularly suitable for high-yield semichemical pulping of softwoods, because the



mitted the addition of jack pine to a balsam-spruce blend without detriment to pulp brightness and other properties. This is in contrast to an otherwise well-known lowering pulp-ing characteristics resulting from an addition of jack pine.

The following table of comparative figures taken from the preceding examples shows the reduction in time for process steps effected by the increase in pressure. Figures illustrative of conventional bisulfite pulping are added for comparison.

| Cooking Stages                   | (Batch type) | AFB<br>(Continuous type) | BSNa<br>Conventional |
|----------------------------------|--------------|--------------------------|----------------------|
| <b>Alkali Impregnation Stage</b> |              |                          |                      |
| Time, minutes                    | 90           | 2                        | none                 |
| Pressure, max., p.s.i.g.         | 100          | 200                      | —                    |
| <b>Bisulfite Cooking Stage</b>   |              |                          |                      |
| Time to max. temp., hrs.         | 6:00         | 1:23                     | 6:00                 |
| Time at max. temp., hrs.         | 0:30         | 1:00                     | 0:40                 |
| Pressure, max., p.s.i.g.         | 100          | 200                      | 85                   |
| Temperature, max., °C.           | 155          | 155                      | 160                  |
| Total Cooking time, hrs.         | 8:00         | 2:25                     | 6:40                 |
| Pulp Yield, %                    | 73.0         | 73.4                     | 73.2                 |

The large reduction in cooking times makes it possible to obtain the previously described advantages of the AFB batch cooking process in a continuous pulping operation.

For more positive pH control in continuous cooking, the SO<sub>2</sub> injected into the digester may be replaced by a solution of bisulfite (containing excess SO<sub>2</sub>). Part of this is made to flow countercurrently to the alkali-treated chips, displacing alkali and leaving the chips impregnated with bisulfite. The alkalized bisulfite solution is withdrawn from the digester and

regenerated with SO<sub>2</sub> in an absorption tower for subsequent reuse. A process embodying these features will form the sub-ject of a further application.

What is claimed is:

1. A process for making pulps of increased pulp yield, high unbleached brightness and high fibrability from coniferous wood, comprising impregnating the wood with an alkaline solution containing not more than about 2 percent by weight of formaldehyde at a pH of about 12.5 at a temperature not exceeding about 100° C. and a pressure between about 100 and about 300 p.s.i.g., draining the solution from the wood, adding liquid or aqueous SO<sub>2</sub> so as to obtain a bisulfite cooking condition, and cooking to obtain maximum pH between about 2.9 and about 4.
15. 2. The process of claim 1 wherein the alkaline solution is a mixture of hydroxide and carbonate.
3. A process as in claim 1 wherein the maximum pH is 2.9.
4. A process as in claim 1 wherein the maximum pH is 3.
5. The process of claim 1 wherein the alkaline impregnation is carried out for about 90 minutes at a temperature not exceeding about 50° C. and a pressure of about 100 p.s.i.g. is em-ployed.
20. 6. A process of claim 1 wherein a short alkaline impregna-tion of about 2 minutes is carried out at about 200 p.s.i.g. pres-sure at a temperature not exceeding about 100° C.
7. The process of claim 1 wherein SO<sub>2</sub> is injected in liquid or aqueous form after draining of the impregnation liquor and the cook is carried out in a vapor or trickle phase.
30. 8. A process as in claim 1 wherein the impregnation pH is not lower than 12.6

\* \* \* \* \*